

# United States Patent Office

2,902,472

Patented Sept. 1, 1959

1

2,902,472

## PRODUCTION OF DICYANDIAMIDE TRIETHYLENE TETRAMINE FORMALDEHYDE CONDENSATE

Alton A. Cook, Glen Ridge, and Ira Sapers, Newark, N.J., assignors to Arkansas Company, Inc., Newark, N.J., a corporation of New York

No Drawing. Application March 8, 1955  
Serial No. 493,046

1 Claim. (Cl. 260—70)

The present invention relates to products and processes for treatment of fabrics dyed with direct dyestuffs to increase the fastness of the dyestuffs to wet treatments including laundering.

It is among the objects of the present invention to provide pretreatments and aftertreatments and the assistants for such purposes for application to dyed fabrics which will render such dyed fabrics fast to hot alkaline treatments with little or no change in color value.

It is a further object of this invention to provide textile assistant compositions which are readily and practically employed in the treatment of textile fabrics both before and after dyeing.

Another object is to provide novel textile assistant compositions which when utilized in a finishing bath will impart to dyed fabrics substantial resistance to alkaline treatments at a wide range of temperatures with a minimum of deleterious effect upon the fabric.

Still further objects and advantages will appear in the more detailed description set forth below, it being understood, however, that this more detailed description is given by way of illustration and explanation only and not by way of limitation, since various changes therein may be made by those skilled in the art without departing from the scope and spirit of the present invention.

In accomplishing the above objects it has been found highly satisfactory to treat the fabric, after it has been dyed, with a condensation product of a nitrogenous compound such as dicyandiamide, acrylamide, urea or guanidine on the one hand; low molecular polyethylene polyamines on the second hand; and formaldehyde on the third hand.

Some of the polyethylene polyamines which may be used are triethylene tetramine (preferred), diethylene triamine and ethylene diamine.

This condensation product for the use of the invention is preferably formed in the presence of a water soluble, low molecular weight aliphatic acid, such as propionic, lactic, acetic or formic, at a controlled pH of 4.5 to 6.0 at a controlled temperature range of 75°-85° C.

The organic acid should have 1 to 6 carbon atoms and the acid may contain from 0 to 3 hydroxy groups and from 1 to 3 carboxy groups. Less preferred are citric, tartaric, maleic, succinic or fumaric acid.

In the present invention particular care is used to control the pH of the reaction so as to keep it on the acid side at all times and the preferred pH range is 4.8 to 5.5 with a broader range of 4.5 to 6.5.

An important feature of the present invention resides in the fact that there is no formation of insoluble matter during the reaction carried out by our process, even after standing for several months at ordinary room temperatures (70° to 90° F.).

In the present invention the degree of polymerization is controlled so that a water soluble condensate of relatively low molecular weight is formed, without giving rise to side reactions which may yield products of relatively high molecular weight and low water solubility.

2

To give specific examples of this invention:

### Example No. 1

- 67.0 parts by weight dicyandiamide (about  $\frac{1}{2}$  mol)  
5 29.0 parts by weight triethylene tetramine (about  $\frac{1}{2}$  mol)  
110.0 parts by weight formaldehyde 37% (about  $1\frac{1}{3}$  mol)  
30.0 parts by weight acetic acid 100% (about  $\frac{1}{2}$  mol)  
10 40.0 parts by weight water

A reactor was charged with dicyandiamide and triethylene tetramine. Acetic acid dissolved in water was then added, and finally the formaldehyde was added. The mixture was then heated slowly to 60° C., whereupon the temperature jumped automatically to 90° C.

The mixture was then cooled to 82° C., and maintained at 78° to 82° C. for about two hours.

The mixture was then rapidly cooled to room temperature.

20 20 A cotton muslin, dyed with 2% Direct Brown BRL (prototype 47), was aftertreated for 20 minutes at 160° F. at a 30 to 1 ratio bath with 6.5% of this reaction product based on the weight of the fabric.

25 Cloth was then rinsed thoroughly and dried.

The aftertreated cloth is fast to bleeding in water. The aftertreated cloth was subjected to a 0.5% soap solution for 30 minutes at 120° C. in a launderometer with 10 steel balls.

30 This last-mentioned treatment is hereafter referred to as a #2 AATCC test.

There is no loss in color and the white cloth was only slightly stained.

### Example No. 2

- 35 84 parts by weight dicyandiamide (about 1 mol)  
15 parts by weight triethylene tetramine (about  $\frac{1}{10}$  mol)  
110 parts by weight formaldehyde 37% (about  $1\frac{1}{3}$  mol)  
14 parts by weight formic acid 90% (about  $\frac{1}{4}$  mol)  
46 parts by weight water

40 A reactor was charged with the dicyandiamide, the triethylene tetramine and the formic acid. The water was added and then the formaldehyde. The mixture was raised slowly to 75° C. Then the heating was stopped and the temperature jumped automatically to 82° C.

45 For about two hours the temperature was maintained at 78° to 82° C., with constant stirring.

The viscous, aqueous solution was cooled rapidly to room temperature.

50 A cotton fabric dyed with Direct Red B (Color Index 419) was aftertreated at 30 to 1 bath ratio for 20 minutes at 160° F. with 6.5% of this reaction product based on the weight of the fabric, and then rinsed with hot water and finally with cold water. The fabric was then subjected to a #2 AATCC washing test.

55 Compared with untreated cloth, it lost only little of the original color.

### Example No. 3

- 84 parts by weight dicyandiamide (about 1 mol)  
34 parts by weight diethylene triamine (about  $\frac{1}{3}$  mol)  
60 164 parts by weight lactic acid 44% (about 0.8 mol)  
110 parts by weight formaldehyde 37% (about  $1\frac{1}{3}$  mol)

65 The lactic acid was added to the dicyandiamide and diethylene triamine. Then the formaldehyde was added and heated under stirring to 70° C.

68 The temperature automatically jumped to 88° C. The mixture was cooled to 80° C. and maintained at 78° to 82° C. for about 2 hours.

70 The reaction product was then cooled rapidly to room temperature.

70 Cotton cloth dyed with 2% Direct Brown BRL (Prototype 49) was aftertreated with 6.5% of the reaction

product based on the weight of the fabric, according to procedure in Example No. 2.

This treatment increased considerably the resistance of the dyeing to bleeding and washing at 120° F.

*Example No. 4*

84 parts by weight dicyandiamide (about 1 mol)  
60 parts by weight acetic acid 100% (about 1 mol)  
75 parts by weight triethylene tetramine (about ½ mol)  
110 parts by weight formaldehyde 37% (about 1½ mol)  
60 parts by weight water

The dicyandiamide was added to the acetic acid, which was diluted with water. The triethylene tetramine was then added and finally the formaldehyde. The mixture was then heated at 78° to 82° C. for about 3 hours and then cooled to room temperature.

Cotton cloth dyed with 1½% Direct Blue Green BL (Color Index 470) was aftertreated with 4.5% of the reaction product based on the weight of the fabric, plus 0.5% acetic acid—56% strength—for 20 minutes at 180° F. The cloth was then thoroughly rinsed and dried.

This treatment made the dyeing resistant to #2 AATCC washing.

*Example No. 5*

84 parts by weight dicyandiamide (about 1 mol)  
15 parts by weight triethylene tetramine (about ¼ mol)  
30 parts by weight acetic acid, glacial (about ½ mol)  
163 parts by weight formaldehyde 37% (about 2 mol)  
40 parts by weight water

The acetic acid diluted in water was added to a mixture of dicyandiamide and triethylene tetramine in a vessel, and then the formaldehyde was added.

The mixture was treated for 1½ hours at 78° to 82° C.

Cotton cloth dyed with 2% Direct Blue FF (Color Index 518) was aftertreated for 20 minutes at 160° F. with 8% of this product.

This treatment rendered the dyeing resistant to the #2 AATCC washing.

*Example No. 6*

67.0 parts by weight dicyandiamide (about ¾ mol)  
14.0 parts by weight acrylamide (about ½ mol)  
21 parts by weight diethylene triamine (about ½ mol)  
40.0 parts by weight acetic acid, glacial (about ¾ mol)  
123.0 parts by weight formaldehyde 37% (about 1½ mol)  
50.0 parts by weight water

The reaction procedure was the same as in Example No. 5.

Cotton cloth dyed with 2% Direct Brown BRL (Prototype 49) was aftertreated with 6.4% of the reaction product based on the weight of the fabric, using the same procedure as in Example No. 5.

This treatment rendered the dyeing fast to bleeding in water and to #2 AATCC washing.

*Example No. 7*

67.0 parts by weight dicyandiamide (about ¾ mol)  
38 parts by weight triethylene tetramine (about ¼ mol)  
12.0 parts by weight urea (about ½ mol)  
110 parts by weight formaldehyde 37% (about 1½ mol)  
45 parts by weight acetic acid, glacial (about ¾ mol)  
60.0 parts by weight water

The reaction procedure was the same as in Example 5.

Cotton cloth dyed with 2% Direct Brown BRL (Prototype 49) was aftertreated with 6.8% of the reaction product based on the weight of the fabric, according to the procedure used in Example No. 5.

This treatment rendered dyeing fast to bleeding in water and to #2 AATCC washing.

*Example No. 8*

63.0 parts by weight dicyandiamide (about ¾ mol)  
47.0 parts by weight guanidine carbonate (about ¼ mol)

20 parts by weight ethylene diamine 77% (about ¼ mol)  
60.0 parts by weight acetic acid, glacial (about 1 mol)  
122.0 parts by weight formaldehyde 37% (about 1½ mol)

5 40.0 parts by weight water

The acetic acid, dissolved in water, was slowly added to mixture of dicyandiamide, guanidine carbonate and ethylene diamine, and then formaldehyde was added. The temperature was slowly raised to 80° C. under constant stirring. The mixture was treated at 80° to 85° C. for 1¾ hours.

Cotton cloth dyed with 2% Direct Brown BRL (Prototype 47) was aftertreated for 20 minutes at 180° F. with 7.0% of the reaction product based upon the weight of the fabric. The cloth was then washed and dried.

This treatment made the dyeing quite fast to bleeding in water and to #2 AATCC washing.

*Example No. 9*

84 parts by weight dicyandiamide  
39 parts by weight ethylene diamine 77% (about ½ mol)  
163 parts by weight formaldehyde 37% (about 2 mol)  
51 parts by weight formic acid 90% (about 1 mol)  
60 parts by weight water

Formic acid, diluted with water, was added to mixture of dicyandiamide and ethylene diamine with cooling and stirring. Then the formaldehyde was added under the same conditions. The temperature was slowly raised to 80° C. and maintained for 5 hours.

Cotton cloth, dyed with Direct Blue FF (Color Index 518) was aftertreated with 8% of the reaction product based on the weight of the fabric for 20 minutes at 180° F.

The resultant treatment makes the dyeing more resistant to #2 AATCC washing.

Variations in the above formula are permissible but the proportion of formaldehyde should always be in the range of 1 to 2 mols to each mol of dicyandiamide or other nitrogenous component.

Variations are permissible in the type and amount of acid used with the restrictions that the acid must be a low molecular weight water soluble organic acid having 1 to 6 carbon atoms.

The product of this invention is chiefly recommended for use as an aftertreatment on fabrics dyed with direct dyestuffs to increase the fastness of hot alkaline treatments or launderings.

In this application the amount of the product used depends upon the depth of shade of the fabric in question, usually from 2% to 10% on the weight of the material together with a small amount of water soluble organic acid, if desired.

In some cases the compositions of this invention may be used as a pretreatment and in this way acts as a mordant for the dyestuffs. Such treatments are usually not as effective as aftertreatments in regard to resistance to bleeding and laundering.

The products of this invention may also be used in connection with copper salts, such as copper chloride, and/or copper acetate, in dyeing procedures when dyes selected from a group suitable for use with copper salts are employed. As a result of such procedures, better wash-fastness is usually obtained as well as improved light-fastness.

In general, in the above examples there was always one or more mols of formaldehyde for each mol of nitrogenous organic base and the molar proportion of dicyandiamide always exceeded the molar proportion of the polyamine.

In general the following ingredients were employed and condensed together:

(a) A nitrogenous base compound, preferably dicyandiamide and less preferably urea, guanidine, acrylamide and

thiourea in amounts of  $\frac{1}{2}$  to 2 mols and preferably in amount of 1 mol.

(b) A polyalkylene polyamine such as triethylene tetraamine, diethylene triamine and ethylene diamine in amounts of  $\frac{1}{8}$  to  $\frac{1}{2}$  mol and preferably  $\frac{1}{4}$  mol.

(c) Formaldehyde in amount of  $\frac{1}{2}$  to 4 mols and preferably 1 to 2 mols.

Where it is desired to use anhydrous conditions, or a waterless system, a paraformaldehyde may be used in the presence of methyl alcohol, which functions as a methylating agent.

The molar proportions above are employed under these conditions except that the methyl alcohol is used in molar proportion ranging from  $\frac{1}{2}$  to 2 mols for each free  $\text{NH}_2$  group.

The basic reaction that takes place is a combination in the fiber itself between the cationic condensation product of the two or three nitrogenous compounds above specified and the formaldehyde together with anionic dyestuff and this combination in the actual textile fiber is highly resistant to washing tests.

Where the acid is used in aqueous condition, it is preferably added in water solution with cooling to the mixed nitrogenous bases.

Following the addition of the acid, the formaldehyde in aqueous solution is also added slowly with cooling.

As a final operation, the reaction mixture is heated.

As many changes could be made in the above process for aftertreatment of dyed fabrics due to improve the wash fastness of dyes, and many widely different embodiments of this invention could be made without departing from the scope of the claim, it is intended that all matter con-

tained in the above description shall be interpreted as illustrative and not in a limiting sense.

Having now particularly described and ascertained the nature of the invention, and in what manner the same is to be performed, what is claimed is:

Process for the production of a condensation product suitable for the treatment of fabrics dyed with a direct dyestuff to increase the fastness properties of said dyestuff, which comprises heating to a temperature of  $60^{\circ}$  C. a mixture of about  $\frac{1}{8}$  mol of dicyandiamide, about  $\frac{1}{6}$  mol of triethylene tetraamine and about  $1\frac{1}{3}$  mols of formaldehyde 37%, the reaction mixture also containing water and acetic acid in an amount sufficient to maintain the pH of said reaction mixture within a range of about 4.5 to 6, and immediately after the initiation of the reaction maintaining the temperature of the reaction mixture for the balance of the course of the reaction at  $75$  to  $85^{\circ}$  C., the temperature at no time being allowed to exceed about  $90^{\circ}$  C., the time of the reaction being from  $1\frac{1}{2}$  to 5 hours.

#### References Cited in the file of this patent

#### UNITED STATES PATENTS

|           |          |                |
|-----------|----------|----------------|
| 2,214,067 | Petersen | Sept. 10, 1940 |
| 2,364,726 | Landolt  | Dec. 12, 1944  |
| 2,366,129 | Rust     | Dec. 26, 1944  |
| 2,405,863 | Treboux  | Aug. 13, 1946  |
| 2,622,075 | Hemmi    | Dec. 16, 1952  |
| 2,631,920 | Albrecht | Mar. 17, 1953  |
| 2,649,354 | Hemmi    | Aug. 18, 1953  |